

Aug. 7, 1934.

J. G. CAPSTAFF  
MATERIAL AND PROCESS FOR MAKING MULTICOLOR  
SUBTRACTIVE PHOTOGRAPHIC PRINTS  
Filed Nov. 12, 1931

1,969,452

*Fig.1.*



*Fig.2.*



Inventor:  
*John G. Capstaff,*

By *Newton M. Perrine*

Attorney

Patented Aug. 7, 1934

1,969,452

# UNITED STATES PATENT OFFICE

1,969,452

## MATERIAL AND PROCESS FOR MAKING MULTICOLOR SUBTRACTIVE PHOTOGRAPHIC PRINTS

John G. Capstaff, Rochester, N. Y., assignor to Eastman Kodak Company, Rochester, N. Y., a corporation of New York

Application November 12, 1931, Serial No. 574,534

10 Claims. (Cl. 95—2)

This invention relates to color photography and more particularly to a material and process for making multi-color subtractive photographic prints in which several component color images are formed on each side of a double coated film. The invention describes a new type of film to be used for such a process.

In processes previously described for producing a plurality of color images on a double coated film, such as for example a process involving one component image on one side and two on the other, it has been necessary to carry out several printing and drying operations. It is one of the objects of my invention to reduce the number of separate printing and intermediate drying operations required in such a process.

The new film which I use consists of a transparent support coated on each side with a photographic emulsion of the positive type, one or both of the emulsion layers containing a water soluble dye to limit the penetration of the actinic light rays, and a layer of water-proof varnish being coated over the emulsion on one side of the film. This water-proof varnish is removable by solution in organic or other solvents or by other suitable means.

Reference is made to the accompanying drawing in which

Figure 1 is a cross section on an enlarged scale of a film made according to my invention.

Figure 2 is a similar cross section of a preferred form of film which I use in my invention.

A transparent support 1 such as a film of cellulose nitrate or cellulose acetate for example, is coated on either side with positive sensitive emulsion 2 and 3 (Figure 1) or 2' and 3' (Figure 2). Over either of these emulsions is placed a very thin coating of a water-proof varnish 4.

In the preferred form of this film (Figure 2), one of the emulsion layers contains a light restraining dye, such a dyed emulsion coating being shown as 2' in Figure 2.

Dyes which are suitable as light restraining dyes to be placed in the emulsion as described are tartrazine, acid yellow, filter K, and naphthol yellow.

For the varnish layer 4 any suitable water-proof varnish which is soluble in a solvent which will not distort the support may be used. An example of such a varnish is the following:

|                        |          |
|------------------------|----------|
| Cellulose-benzyl ether | 150 g.   |
| Benzene                | 1550 cc. |
| Toluene                | 100 cc.  |
| Xylene                 | 400 cc.  |

This coating may be easily removed with benzene.

One of the most advantageous uses of such a film is in the making of a three color subtractive print, by which I will illustrate its use.

The film described is exposed from the one

side through one of the three color component negatives, say the red negative, and from the other side, in register, through another of the component negatives, say the green. These exposures may be made simultaneously or in succession, and by contact or projection.

Let it be assumed that the exposure from the unvarnished side of the film was made through the red filter component negative. The film is then developed by immersion in a developer that produces, in addition to the silver image, an accompanying image of an insoluble blue-green dye. Typical developers are the following:

### Formula I

75

|                             |             |
|-----------------------------|-------------|
| Diethyl p-phenylene diamine | 8 gm.       |
| Sodium sulfite              | 40 gm.      |
| Sodium carbonate            | 60 gm.      |
| Dichloronaphthol            | 1.56 gm. 80 |
| Acetone                     | 44 c. c.    |
| Water                       | 4000 c. c.  |

### Formula II

|                                                          |              |
|----------------------------------------------------------|--------------|
| Sodium carbonate (per 100 g. per l.)                     | 40 c. c. 85  |
| Sodium sulphite                                          | 0.5 g.       |
| p-amino-diethyl-aniline-hydrochloride                    | 1.0 g.       |
| 3,5-dibromo-o-cresol, 50 g. per l. dissolved in 95% alc. | 20 c. c. 90  |
| Water to                                                 | 100 c. c. 90 |

The film is now washed and passed through a solution that converts the silver image to one of a silver salt, such as a solution of potassium ferricyanide and potassium bromide. The silver salts are now removed with a solution of plain sodium thiosulphate, and the film is thoroughly washed in water. It is understood that the above solutions and wash waters act only upon the unvarnished side of the film.

In producing this colored image, as well as the following ones, it is not essential that a color forming developer be used. The image can be produced by any recognized method, as for example, by dye toning. Numerous examples of typical dye-toning processes are to be found in "The Tinting and Toning of Eastman Positive Motion Picture Film," fourth edition, published by Eastman Kodak Co., Rochester, N. Y., 1924. It must however, not be affected by any of the subsequent operations.

I prefer to varnish this first image, as this varnish layer may be advantageously left on during all the following operations and acts as a protective layer for the finished film. This varnishing operation on the first image is carried out after removing the varnish from the other side, the originally varnished side. At this stage the steps, then are (1) The film is passed through (immersed in) a suitable organic sol-

vent, such as benzine, which removes the varnish layer from the undeveloped side of the film. (2) The developed side (first image) is then varnished.

- 5 Let it be assumed that the undeveloped side of the film has been exposed, in the above described printing operation, through the green filter component negative. The film is now developed by immersing in a developer that produces, in addition to the silver image, an accompanying insoluble image of a magento dye. A suitable developer is the following

*Formula III*

|    |                                                                         |     |       |
|----|-------------------------------------------------------------------------|-----|-------|
| 15 | Sodium carbonate 10% aqueous solution                                   | 30  | c. c. |
|    | Sodium sulfite anhydrous                                                | 1   | gm.   |
|    | p-amino dimethyl aniline hydrochloride                                  | 0.2 | gm.   |
| 20 | 1-phenyl-3-methyl-5-pyrazolone 0.2 grams dissolved in 95% ethyl alcohol | 10  | c. c. |
|    | Potassium bromide 10%                                                   | 0.2 | c. c. |
|    | Water to                                                                | 100 | c. c. |

The film is now washed and passed through a solution that converts the developed silver to a salt of silver not susceptible to development without further exposure to light and destroys any remaining latent image. Such a solution is the following.

|    |                  |     |       |
|----|------------------|-----|-------|
| 30 | Ammonium bromide | 24  | grams |
|    | Iodine           | 0.5 | gram  |
|    | Water to         | 500 | c. c. |

This bath is used so that any remaining undeveloped latent image will not develop in the yellow developer without further exposure to light. Otherwise some of the image which should have been magenta will become yellow. The film is now washed and passed through a sensitizing bath, such as for example a 1/2% solution of sodium sulphite.

At this stage, before printing the third image, it is desirable to re-introduce a yellow light restraining dye similar to that originally present in the film. This is necessary to produce the same gamma in the third image as in the other two, and to restrict the depth of this third image to the lower part of the layer in which it is printed from the opposite side. The yellow dye may be conveniently introduced by dissolving about 1/2% of the dye (tartrazine, acid yellow or others) in the 1/2% sodium sulphite sensitizing solution.

After drying, the film is again exposed, through the first developed and fixed side (the originally unvarnished side), to the third color component negative, say the blue, in registry with the first two images. The film is now developed by immersing in a developer that produces, in addition to the silver image, an accompanying image of a yellow color such, for instance, as a mixture of alpha-chlorethylacetate with diethyl para-phenylene diamine. The film is now washed and passed through a solution that converts the silver image to one of a silver salt, such as a solution of potassium ferricyanide and potassium bromide. All the remaining silver salts are now removed with a solution of plain sodium thiosulphate, and the film is thoroughly washed and dried. It now bears the completed three color subtractive print.

The order of introducing the three color images is not essential, although it is preferable that the first introduced image be either blue-green or magenta in order to be transparent to the actinic rays in the second printing. This avoids

the necessity for color sensitizing the film or for printing through filters. Other developers such as those disclosed in the patents to Fischer 1,055,155, March 4, 1913 and 1,102,028, June 30, 1914, and disclosed in "History of Three-Color Photography" by E. J. Wall, published 1925, pages 404 et seq., may be used.

All of the developers and solutions which I use are well known in the art and have been previously described. They form no part of the present invention.

By the process described only two printing operations and one intermediate drying of the film are required to introduce three images.

The special film described may also be used to advantage in the production of two color subtractive prints in which both images are printed at the beginning and the iodine bleach and sulphite sensitizing baths or their equivalents, as well as the third exposure and development, are omitted. It will be apparent that a number of other variations are possible at the different stages.

I consider as included in my invention all variations and equivalents coming within the scope 100 of the appended claims.

What I claim is:

1. A film for a color photographic process in which color component images are formed on each side of a film, comprising a transparent support, at least one sensitive emulsion layer on each side of said support and a thin, easily removable, waterproof coating over one of said sensitive layers.

2. A film for a color photographic process in which color component images are formed on each side of a film, comprising a transparent support, a sensitive emulsion layer on each side of said support, a water soluble dye in one of said emulsion layers to limit the penetration of effective 115 light rays, and a thin coating of a waterproof varnish which is readily removable in suitable solvents over one of said sensitive emulsion layers.

3. In a color photographic process, the steps that comprise printing from color separation 120 negatives upon opposite sides of a film having a sensitive emulsion layer on each surface, one of which layers is covered by a waterproof protective layer, thereby forming in registry latent images in each sensitive layer, transforming one 125 latent image into a color image without affecting the latent image in the layer under the protective coating and then removing the protective coating and transforming the other latent image into a color image.

4. A color photographic process comprising forming different color component latent images in two sensitive layers on opposite sides of the same film, one of said layers being covered by a transparent, waterproof coating, submitting 135 the film to a color forming developer whereby a colored image is formed in the uncovered layer, removing said coating and submitting the film to a different color forming developer whereby an image of different color from the first is 140 formed in the previously protected layer.

5. A color photographic process which comprises the making of three color separation negatives through different color filters, printing from two of said negatives in register upon opposite sides of a film having a sensitive layer on each side and having a waterproof layer over one sensitive layer, thereby forming latent images in each layer, transforming the latent image in the uncovered sensitive layer into a 150

color image, removing the protective coating, transforming the other latent image into a color image, and then forming in one of said layers a color image from the third separation 5 negative.

6. A color photographic process which comprises the making of three color separation negatives through different color filters, printing from two of said negatives in register upon opposite sides of a film having a sensitive layer on each side and having a waterproof layer over one sensitive layer, thereby forming latent images in each layer, transforming the latent image in the uncovered sensitive layer into a color image, removing the protective coating, transforming the other latent image into a color image, resensitizing one of said layers and printing therein a latent image from the third negative and transforming this last named image into a third color image, the three color images being of different colors and each complementary to the color of the filter through which the corresponding negative was taken.

7. A color photographic process which comprises making three color separation negatives through different color filters, printing two of said separation negatives in register upon opposite sides of a positive film having an emulsion layer on each surface and which contains a water soluble light restraining dye in one emulsion layer and has a thin waterproof varnish layer over one of the emulsion layers, developing the film in a color-forming developer, converting the silver image associated with the color image into a silver salt, removing the varnish layer from the undeveloped side of the film, developing the film in a second color forming developer, submitting the film to the action of an oxidizing solution that converts the developed silver to a salt of silver which is not susceptible to development without further exposure to light and destroys any remaining latent image, resensitizing one of the emulsion layers, printing in register in the resensitized layer the third color separation negative, developing the third image so produced in a third color-forming developer, submitting the film to the action of a solution that converts the silver image to a silver salt, and removing all the remaining silver salts.

8. A color photographic process which comprises making three color separation negatives through different color filters, printing two of said separation negatives in register upon opposite sides of a positive film having an emulsion layer on each surface and which contains a water soluble light restraining dye in one emulsion layer and has a thin waterproof varnish layer over one of the emulsion layers, developing the film in a color-forming developer that gives a product complementary in color to that of the filter used in taking the color separation negative which is printed on the unvarnished side of the said positive film, converting the silver image associated with the color image into a silver salt, removing the converted silver salts, removing the varnish layer from the undeveloped side of the film, developing the film in a second color forming developer that produces a product complementary in color to that of the filter used in taking the color separation negative which is printed on the varnished side of the said positive film, submitting the film to the action of an oxidizing solution that converts the developed silver to a salt of silver which is not susceptible to development

without further exposure to light and destroys any remaining latent image, resensitizing one of the emulsion layers, printing in register in the resensitized layer the third color separation negative, developing the third image so produced in a third color-forming developer that gives a product complementary in color to that of the filter used in taking said third color separation negative, submitting the film to the action of a solution that converts the silver image to a silver salt, and removing all the remaining silver salts.

9. A color photographic process which comprises making three color separation negatives through different color filters, printing two of said separation negatives in register upon opposite sides of a double-coated positive film which contains a water soluble light restraining dye in one emulsion layer and has a thin waterproof soluble varnish layer over one of the emulsion layers, developing the film in a color-forming developer, converting the silver image associated with the color image into a silver salt, removing the varnish layer from the undeveloped side of the film, varnishing the developed side, developing the film in a second color forming developer, submitting the film to the action of an oxidizing solution that converts the developed silver to a salt of silver which is not susceptible to development without further exposure to light and destroys any remaining latent image, resensitizing the film, printing in register on the originally unvarnished side the third color separation negative, developing the third image so produced in a third color-forming developer, converting the silver image to a silver salt and removing all the remaining silver salts.

10. A color photographic process which comprises making three color separation negatives through different color filters, printing two of said separation negatives in register upon opposite sides of a double-coated positive film which contains a water soluble light restraining dye in one emulsion layer and has a thin waterproof soluble varnish layer over one of the emulsion layers, developing the film in a color-forming developer that gives a product complementary in color to that of the filter used in taking the color separation negative which is printed on the unvarnished side of the said positive film, converting the silver image associated with the color image into a silver salt, removing the converted silver salt, removing the varnish layer from the undeveloped side of the film, varnishing the developed side, developing the film in a second color forming developer that produces a product complementary in color to that of the filter used in taking the color separation negative which is printed on the varnished side of the said positive film, submitting the film to the action of an oxidizing solution that converts the developed silver to a salt of silver which is not susceptible to development without further exposure to light and destroys any remaining latent image, resensitizing the film and bathing it in a yellow light restraining dye, printing in register on the originally unvarnished side the third color separation negative, developing the third image so produced in a third color-forming developer that gives a product complementary in color to that of the filter used in taking said third color separation negative, converting the silver image to a silver salt and removing all the remaining silver salts.

JOHN G. CAPSTAFF.